

June 11, 1940.

B. S. GREENSFELDER ET AL.

2,204,215

## MANUFACTURE OF MOTOR FUEL

Filed June 15, 1936



Inventors:

Bernard S. Greensfelder  
Russell N. Shiras

By their Attorney: Defender

## UNITED STATES PATENT OFFICE

2,204,215

## MANUFACTURE OF MOTOR FUEL

Bernard Sutro Greensfelder, Martinez, and  
Russell Norman Shiras, Long Beach, Calif., as-  
signors to Shell Development Company, San  
Francisco, Calif., a corporation of Delaware

Application June 15, 1936, Serial No. 85,196

7 Claims. (Cl. 44—9)

This invention relates to improvements in motor fuels and process for manufacturing such fuels from mineral hydrocarbon oils.

Three of the qualities which characterize good 5 gasolines are high antiknock rating, vapor pressure below a certain maximum, and a properly balanced distillation range. The influence of these qualities on the performance of motor fuels in gasoline engines has been the subject of intensive studies during preceding years. Summarizing the results of these studies, it may be stated that, in general, high octane number permits the use of high engine compression ratios which, according to statistics, have risen from an average of 4.5 a few years ago to over 6 to date with a corresponding increase in engine efficiency. Effective volatility, as expressed in terms of vapor pressure and A. S. T. M. distillation, should be such as to combine the lowest possible vapor pressure with a distillation curve which indicates highest volatility index, volatility index being indicative of the percent evaporated at 167° and 284° F. when distilling in accordance with A. S. T. M. method D 86-35. Motor fuels having the above effective volatility requirements insure ease of starting, quick acceleration and freedom from vapor lock. Improvements in the effective volatility of motor fuels can be achieved by lowering the vapor pressure, or the temperature of the 50% evaporated, or both.

The term "octane number" as hereinafter used refers to A. S. T. M. octane number, A. S. T. M. method D 357-34T, provided the number is 100 or below. Octane numbers above 100, are "blending octane numbers," as defined by Sprake et al. in Proceedings of World Petroleum Congress, London 1933, page 170.

The studies of the problem of engine knock have revealed that octane number is a function 40 of the fuel composition, as well as of engine conditions. It was found that octane numbers of an homologous series of hydrocarbons depend upon the number of carbon atoms in their molecules and upon the compactness of their molecular structure, octane numbers rising with numerical decrease and centralization of carbon atoms. Thus the octane number of normal heptane is zero, as compared with —19 for normal octane, while 2-2-3-3 tetramethyl butane, which is one 45 of the isomeric octanes, has an octane number of 130. Double bonds generally contribute to a rise in antiknock value, this rise, however, decreasing with increasing severity of engine conditions. Aromatic and olefinic hydrocarbons, while 50 having excellent antiknock properties in engines operating at relatively low temperatures and speeds, depreciate in octane number at higher engine temperatures and speeds. Moreover, numerous aromatic compounds have comparatively 55 high melting points, which greatly limit

their use at low atmospheric temperatures. Even in summer time, airplane engines have been known to have difficulties when flying at high altitudes, due to obstruction of the fuel lines traceable to frozen aromatic compounds, and olefines are excluded from many aviation gasolines by specifications because of their tendency to form gums.

The effect of tetraethyl lead on the octane 10 number of fuels has also been studied and a factor called the lead susceptibility has been introduced. It has been established that some gasolines show more improvement in octane number for a given addition of tetraethyl lead than do others. This variation in susceptibility was 15 found to be a function of the composition of the fuel, those components which depreciate in octane number at elevated temperatures, in general, being less susceptible to lead. In other words, paraffinic and naphthenic hydrocarbons 20 were found to be much more susceptible to octane number improvement by the addition of tetraethyl lead than olefines and particularly aromatic compounds. Some aromatics are known to possess negative lead susceptibilities.

We have discovered that by close fractionation 25 of suitable low boiling petroleum products, such as naphthas, particularly those obtained from naphthenic base crudes, such as California 30 crudes, natural gasoline, recovery gasoline, etc., two valuable fractions of a boiling range suitable 35 for motor fuels can be isolated, in which non-aromatic hydrocarbons of centralized and/or cyclic structures possessing high octane numbers and lead susceptibilities are concentrated. By 40 blending these fractions with gasolines, blended motor fuels may be produced having antiknock 45 ratings which are not only improvements over those of the unblended gasolines, but which do not depreciate even when these blended fuels 50 are used in engines operating under most severe conditions.

The low boiling fraction of our invention has 55 a boiling range as measured by the 5% and 95% points of the A. S. T. M. distillation method 45 D 86-35, within 40° to 60° C., while the higher boiling fraction has a boiling range as determined 50 in the same manner of within 75° to 95° C., and preferably within 75° to 90° C. These fractions consist of naphthenic and branched paraffinic 55 and/or olefinic hydrocarbons. For convenience and for the reasons hereinafter explained, we shall refer to these two fractions as cyclopentane 60 fraction and cyclo-hexane fraction, respectively. As mentioned hereinbefore, we obtain these fractions by fractional distillation of petroleum or 65 petroleum products, particularly of the type of natural gasoline or similar hydrocarbon mixtures, which may or may not contain aromatic hydrocarbons, and which are preferably derived,

in order to assure proper compositions of these valuable fractions and their substantial yields, from naphthenic base crudes, such as California, Gulf, and some of the West Texas crudes or 5 natural gases accompanying these crudes.

Analyses of many samples of different origins have shown the fraction boiling from 40-60° C. to be characterized by the presence of a considerable amount of cyclopentane, boiling at 50° C. 10 and having an octane number of approximately 130, and relatively small quantities of 2-2 dimethyl butane, 101 octane number, and 2-3 dimethyl butane, 124 octane number. If the original material contains products from a cracking process, this fraction may also contain isomers of hexene which possess relatively high octane numbers. Although, naturally, the concentration of cyclopentane in this fraction varies depending upon its source, we have found that in 15 most cases the concentration of this cyclic hydrocarbon in the properly produced fraction is not below 5% and, frequently, is found to be in excess of about 20%. Whereas these concentrations of cyclopentane are preferred limits, we have found that fractions boiling between about 40-60° C. 20 may still be valuable for blending in gasolines, even though such fractions are deficient in cyclopentane since the branched hexanes contained in the fraction have high antiknock values as afore 25 pointed out. For example, when the fraction is obtained from a cracked distillate, it may contain predominating amounts of branched olefines, such as methyl pentenes, and very small amounts 30 only of cyclopentane.

35 The octane rating of the cyclopentane fraction varies somewhat with its composition within a fairly definite range, that of the preferred type of this fraction being in excess of 80.

The cyclohexane fraction, as the name indicates, includes cyclohexane and also substantial proportions of other hydrocarbons of branched paraffinic and/or olefinic and/or naphthenic types. The concentration of cyclohexane may vary within wide limits, but we prefer to use fractions containing at least 5% cyclohexane, although lower concentrations are permissible, provided the concentration of branched hydrocarbons is such as to assure that the fraction has an octane number of at least 70, the fractions boiling within the range of 75-95° C. having octane ratings below 70 being considered unsuitable for use in blended gasolines in accordance with this invention; an excessive depression of the octane rating of fractions of our preferred boiling range 55 may sometimes be due to relatively high concentrations of some objectionable hydrocarbons, such as 2-methylhexane which has an octane rating of 55. By limiting the upper limit of the boiling range of this fraction to 90° instead of 95° C. 60 certain of these branched heptanes having low antiknock qualities may be eliminated while those boiling below 90° C., all of which possess high antiknock values, are retained in the fraction.

A characteristic of our cyclopentane and cyclohexane fractions is that they are substantially free from aromatic and normal paraffinic hydrocarbons. Although the boiling temperature of benzene (80.2° C.) is within the boiling range of our cyclohexane fraction, this aromatic hydrocarbon is excluded therefrom in the course of fractional distillation due to the known fact, that the vapor pressure relations of benzene and n-hexane cause their nearly complete removal from fractions boiling at temperatures above 75° C. 70

75 The mixture of these two hydrocarbons is distilled

with other hydrocarbons in the boiling range from 60° C. to 75° C. and, therefore, is excluded from both our fractions.

While in the foregoing we have described the cyclopentane and cyclohexane fractions as boiling within the range of 40 to 60° C. and 75 to 95° C., respectively, we do not wish to include in these terms a single substantially pure individual hydrocarbon boiling within one or the other of these ranges, but wish to designate by these terms fractions produced by fractional distillation of hydrocarbon oils of longer boiling ranges. These fractions are preferably prepared so as to have their A. S. T. M. 10% and 90% temperatures separated by at least about 5° C., both temperatures being 15 within the stated ranges.

If the fractions contain objectionable sulfur compounds, unstable unsaturated compounds of the type of diolefines, etc., they may be treated with chemicals or other refining agents such as 20 alkali, "doctor" solution, sulfuric acid, clay, etc.

In the attached drawing, a flow diagram illustrates a method, by which the two desired fractions may be separated from a mixture containing them, and by which the remaining fractions are utilized to produce either further quantities of the desired fractions, or antiknock gasoline with which the desired fractions may be blended, thus further improving its antiknock rating and/or volatility. Vapors of natural gasoline or 30 other suitable mineral oil, are introduced from a source not shown through line 1 into fractionating column 2, from which an overhead vapor boiling below 90° C. is removed through vapor line 3, and a bottom stream, boiling above 90° C., 35 through line 4. The vapors from line 3 are discharged into fractionator 5 in which they are separated into a bottom fraction boiling between 75° and 90° C., and an overhead vapor fraction boiling below 75° C. The 75/90° C. fraction passes through conduit 6 to tank 7. The vapor fraction boiling below 75° C. is conducted through line 8 to fractionator 9 in which it is separated into a bottom fraction boiling between 60° C. and 75° C. which is withdrawn through line 10, and a vapor fraction boiling below 60° C. The latter fraction passes through vapor line 11 to fractionator 12, in which it is separated into a bottom fraction boiling between 40° C. and 60° C., which is conducted through line 13 to tank 14, and an overhead product boiling below 40° C. which passes through lines 15 and 16 into manifold 17 where it joins the bottom streams from lines 4 and 10 from the fractionators 2 and 9, respectively. The combined streams are now forced by pump 18 in line 19 through coil 20 in furnace 21, in which they are heated under superatmospheric pressure, if desired, to a cracking or reforming temperature. The cracked or reformed product now enters through line 22 into fractionator 23, which 55 may consist of a system of fractionating columns, in which they are separated into at least 3 fractions: a normally gaseous fraction which escapes through overhead line 24 and goes to an absorption plant not shown; a gasoline type fraction, 60 which is withdrawn through side line 25; and a tarry bottom fraction which is removed through bottom line 26. A tar-free fraction heavier than gasoline may be produced which flows through side conduit 27 and is recirculated through the heating coil 20 by pump 18 in line 19 to be re-cracked.

The gasoline fraction in line 25 may be conducted through line 28 into fractionator 2 to be recirculated through the fractionating system 75

comprising the fractionators 2, 5, 8, 12, for the production of additional cyclopentane and cyclohexane fractions. Or it may be taken through line 29 to gasoline tank 30. On its way to tank 30 this gasoline may be chemically treated, in a treating plant not shown, in order to desulfurize and/or render it storage stable.

The cyclohexane and cyclopentane fractions in tanks 7 and 14, respectively, may be conducted through lines 31, 29, and 32, 29, respectively, to blending tank 30 for the production of blended gasoline of desired specifications.

The overhead fraction boiling below 40° C. from fractionator 12 and line 15, instead of being passed through line 16 as described, may be conducted through line 33 into fractionator 34, in which normal pentane is withdrawn as the bottom product through line 41 and manifold 17 to go to the reforming unit; and an overhead vapor boiling below 35° C. consisting of isopentane and lighter hydrocarbons which is transferred through line 35 to stabilizer 36 in which isopentane is separated from the lighter hydrocarbons. The latter pass through lines 37 and 24 to the absorption plant not shown, and the isopentane is transferred through line 38 to tank 39. If desired, isopentane may be introduced into the blended gasoline in tank 30 by conducting it through lines 40 and 29. Portions of overhead products from the columns 23 and/or 36 may be recirculated through the cracking coil 28 together with normally liquid hydrocarbons from line 27 and be caused to polymerize or condense therewith.

While the described cyclopentane and cyclohexane fractions have proven to be excellently suited for blending with motor gasolines, their use is not restricted to this. The fractions alone or in combination with each other have the properties of motor fuels for general as well as special purposes. Mixtures of the two fractions may produce aviation gasolines which meet the most exacting demands with regard to volatility, knock rating, and freezing point.

The cyclopentane fraction finds a further application in the manufacture of low vapor pressure gasolines by replacing aliphatic pentanes and lighter hydrocarbons. Thus, by substantially removing aliphatic pentanes and lighter hydrocarbons from a motor gasoline, whereby the vapor pressure of the gasoline is lowered substantially below normal, and then replacing the removed fractions with cyclopentane fraction, a gasoline can be produced having a higher effective volatility and volatility index and a lower vapor pressure and vapor lock tendency than the original motor gasoline. Instead of depentanized gasoline base, a debutanized gasoline having a subnormal volatility can be markedly improved by being blended with a sufficient quantity of the cyclopentane fraction to result in a blend having volatility of normal gasoline. The antiknock rating may be considerably raised by this substitution, and may further be improved by incorporating an effective quantity of the cyclohexane fraction, the improvement being particularly noticeable where the octane number of the original gasoline is below 70.

The proportions of the two fractions required for blending with existing motor gasolines cannot be specified with any degree of accuracy. However, in studying a large number of gasolines, that is, hydrocarbon mixtures boiling between about 30° C. and 200° C. and produced by frac-

tional distillation of petroleum crudes or their fractions, as well as of cracked or reformed distillates, or obtained by blending of straight run and cracked petroleum fractions, alone, or with hydrogenated or synthetic hydrocarbon products, we have found that the concentrations of the cyclopentane and cyclohexane fractions in such gasolines rarely exceed about 8% and about 15% respectively. By adding our cyclopentane and/or cyclohexane fractions to such gasolines, we increase their content of these fractions substantially beyond normal concentrations, which enables us to produce gasolines of markedly superior quality.

Aviation gasolines of very good quality are produced by blending our cyclopentane and cyclohexane fractions, alone, without the addition of a third hydrocarbon component, 1 to 5 parts of the lighter fraction in 10 parts of the blend being required to meet specifications for this type of motor fuel. If the vapor pressure specifications permit, isopentane may be added to the blended gasoline, isopentane having a blending octane number of above 90. The presence of isopentane is not only beneficial to the antiknock rating, but it improves the starting qualities of gasolines, a property which is of great importance in gasolines used in cold weather.

The following examples illustrate our invention:

#### Example 1

A blend is prepared of 70% by volume of a debutanized gasoline base of the properties shown below, with 20% of a cyclopentane fraction and 10% of a cyclohexane fraction. To 80 volume percent of the resulting blend 20% of an isopentane fraction is subsequently added.

|                            | Gasoline base | Blended gasoline, 70% base, 20% cyclopentane frac., 10% cyclohexane frac. | 80% blended gasoline 20% isopentane frac. | Regular gasoline | 40 |
|----------------------------|---------------|---------------------------------------------------------------------------|-------------------------------------------|------------------|----|
| A. S. T. M. dist. I. B. P. | 77            | 48                                                                        | 40                                        | 42               |    |
| 5%                         | 85            | 58                                                                        | 50                                        | 50               |    |
| 10%                        | 90            | 65                                                                        | 58                                        | 70               |    |
| 50%                        | 135           | 123                                                                       | 120                                       | 130              |    |
| 90%                        | 190           | 189                                                                       | 189                                       | 189              |    |
| 95%                        | 201           | 201                                                                       | 201                                       | 200              |    |
| F. B. P.                   | 207           | 207                                                                       | 206                                       | 206              | 50 |
| Reid V. P. at 100° F.      | 2.1           | 4.2                                                                       | 8.5                                       | 8.6              |    |
| Octane No.                 | 50            | 61                                                                        | 68                                        | 56               |    |

#### Example 2

An aviation gasoline consisting of 3 parts of a cyclopentane fraction and 7 parts of a cyclohexane fraction has the following properties:

|                            | Cyclopentane fraction | Cyclohexane fraction | Blend, 3 pts. cyclopentane, 7 pts. cyclohexane | Regular aviation gasoline | 60 |
|----------------------------|-----------------------|----------------------|------------------------------------------------|---------------------------|----|
| A. S. T. M. dist. I. B. P. | 41                    | 75                   | 43                                             | 47                        |    |
| 5%                         | 42                    | 76                   | 48                                             | 65                        |    |
| 10%                        | 44                    | 77                   | 52                                             | 75                        |    |
| 50%                        | 50                    | 85                   | 79                                             | 94                        |    |
| 90%                        | 68                    | 92                   | 91                                             | 114                       |    |
| 95%                        | 59                    | 93                   | 93                                             | 128                       |    |
| E. B. P.                   | 60                    | 96                   | 96                                             | 140                       |    |
| Reid V. P. at 100° F.      | 11.2                  | 2.7                  | 5.6                                            | 5.2                       |    |
| Octane No.                 | 90                    | 75                   | 80                                             | 73                        | 70 |

#### Example 3

An aviation gasoline is prepared by blending 4 parts of a depentanized aviation gasoline base.

with 3 parts of a cyclopentane fraction and 3 parts of a cyclohexane fraction.

| 5  | Aviation gasoline base         | Blended aviation gasoline, 4 parts base, 3 parts cyclopentane frac., 3 parts cyclohexane frac. | Regular aviation gasoline |
|----|--------------------------------|------------------------------------------------------------------------------------------------|---------------------------|
| 10 | A. S. T. M. dist. I. B. P. . . | 77                                                                                             | 42                        |
|    | 10%-----                       | 86                                                                                             | 52                        |
|    | 50%-----                       | 96                                                                                             | 80                        |
|    | 90%-----                       | 114                                                                                            | 110                       |
|    | F. B. P.-----                  | 139                                                                                            | 137                       |
|    | Reid V. P. at 100° F-----      | 1.6                                                                                            | 5.0                       |
|    | Octane No.-----                | 70                                                                                             | 78                        |
|    |                                |                                                                                                | 73                        |

15

We claim as our invention:

1. A gasoline-type motor fuel of normal vapor pressure consisting essentially of a blend of a depentanized portion of a gasoline distillate having a subnormal vapor pressure and a quantity of a cyclopentane fraction obtained by distillation of petroleum oil containing said fraction consisting essentially of naphthenic and branched chain aliphatic hydrocarbons and being substantially free from aromatic and normal paraffinic hydrocarbons.
2. A gasoline-type motor fuel of normal vapor pressure consisting essentially of a blend of a depentanized portion of a gasoline distillate having a subnormal vapor pressure and a quantity of a mineral oil fraction having a boiling range not exceeding 40° C. to 60° C. consisting essentially of naphthenic and branched chain aliphatic hydrocarbons and being substantially free from aromatic and normal paraffinic hydrocarbons.
3. A gasoline-type motor fuel of normal vapor pressure consisting essentially of a blend of a depentanized portion of a gasoline distillate having a subnormal vapor pressure and a quantity of a cyclopentane fraction obtained by distillation of petroleum oil containing said fraction consisting essentially of naphthenic and branched chain aliphatic hydrocarbons and being substantially free from aromatic and normal paraffinic hydrocarbons, said quantity being from 1 to 5 parts in 10 parts of the blend.
4. A gasoline-type hydrocarbon mixture of

normal vapor pressure and volatility index consisting essentially of a blend of a depentanized portion of a gasoline distillate having a subnormal vapor pressure and volatility index, and a quantity of a mixture of cyclopentane and cyclohexane fractions, said fractions obtained by distillation of petroleum oil containing said fractions consisting essentially of naphthenic and branched chain aliphatic hydrocarbons and being substantially free from aromatic and normal paraffinic hydrocarbons.

5. A gasoline-type hydrocarbon mixture of normal vapor pressure and volatility index consisting essentially of a blend of a depentanized portion of a gasoline distillate having a subnormal vapor pressure and volatility index and a quantity of a mixture of two mineral oil fractions having boiling ranges not exceeding 40° C. to 60° C. and 75° C. to 95° C. respectively, said fractions consisting essentially of naphthenic and branched chain aliphatic hydrocarbons and being substantially free from aromatic and normal paraffinic hydrocarbons.

6. A gasoline-type hydrocarbon mixture of normal vapor pressure and volatility index consisting essentially of a blend of a depentanized portion of a gasoline distillate having a subnormal vapor pressure and volatility index and a quantity of a mixture of two mineral oil fractions having boiling ranges not exceeding 40° C. to 60° C. and 75° C. to 90° C. respectively, said fractions consisting essentially of a naphthenic and branched chain aliphatic hydrocarbons and being substantially free from aromatic and normal paraffinic hydrocarbons.

7. A gasoline-type motor fuel of normal vapor pressure consisting essentially of a blend of a gasoline distillate substantially free from C<sub>5</sub> and lighter hydrocarbons having a subnormal vapor pressure and a quantity of a cyclopentane fraction obtained by distillation of petroleum oil containing said fraction consisting essentially of naphthenic and branched chain aliphatic hydrocarbons and being substantially free from aromatic and normal paraffinic hydrocarbons.

BERNARD SUTRO GREENSFELDER.  
RUSSELL NORMAN SHIRAS.